

# UNITED STATES PATENT OFFICE.

ALFRED JAMES BAILEY, OF BRIXTON, LONDON, ENGLAND.

## PACKING FOR STUFFING-BOXES.

1,158,770.

Specification of Letters Patent.

Patented Nov. 2, 1915.

No Drawing.

Application filed February 17, 1915. Serial No. 8,956.

To all whom it may concern:  
Be it known that I, ALFRED JAMES BAILEY, residing at 42 Appach road, Brixton, London, England, have invented certain new and useful Improvements in Packing for Stuffing-Boxes; and I do hereby declare the following to be a full, clear, and exact description of the invention, such as will enable others skilled in the art to which it appertains to make and use the same.

This invention relates to compressible metallic packing compositions, and more especially to packing compositions in which a readily fusible metal, white metal for example, is mixed in a melted state with pulverized talc or similar substance such as powdered graphite, to produce a metal powder to which other suitable substances are added, for example small quantities of asbestos fiber, flaky graphite and fat to produce a plastic lubricant packing.

Such metallic packing compositions as heretofore composed possess little or no resiliency and the object of the present invention is to increase the efficiency of the packing by imparting greater resiliency thereto, while leaving its durability and imperviousness unimpaired.

With the above object in view my invention consists in adding a small quantity of powdered cork to the packing composition. By the term powdered cork I mean cork reduced to a fineness approximating to that of flour.

I have found that a mixture in the following proportions by weight gives good results:

|                     |    |      |
|---------------------|----|------|
| White metal         | 28 | lbs. |
| Powdered talc       | 1  | "    |
| Powdered graphite   | 1½ | "    |
| Powdered cork       | ½  | "    |
| Fat (engine tallow) | 1½ | "    |
| Carded asbestos     | 1  | "    |

In another composition the proportion of cork employed is two pounds, the propor-

tions of the other ingredients remaining the same as given in the preceding example, but the proportions may of course be varied according to requirements, and the powdered talc is in some cases entirely replaced by powdered graphite.

In the manufacture of the packing the metal is melted and while in the molten state the powdered talc, or powdered graphite or both these substances are added and mixed thoroughly therewith so that on the cooling of the mixture a metallic powder is produced. The powdered cork and other ingredients are added to the metallic powder to form a plastic and resilient packing material.

The natural mineral lubricant, such as talc or graphite, is used so that the metal may be pulverized. Other approved mineral lubricants may be used, but graphite is preferred as it can be used for all purposes, whereas talc unfits the packing for use in connection with pumps. Other kinds of fat besides tallow may be used. Other kinds of fibrous material besides asbestos may also be used, but carded asbestos is preferred. The cork must be in the form of flour or powder, as when granulated cork is used charring takes place and the packing is spoiled.

What I claim is:

1. A packing composition, comprising a pulverized metal mixed with a natural mineral lubricant, fat, fibrous material, and powdered cork.

2. A packing composition, comprising a pulverized metal mixed with a natural mineral lubricant, fat, carded asbestos, and powdered cork.

In testimony whereof I affix my signature, in presence of two witnesses.

ALFRED JAMES BAILEY.

Witnesses:

ARTHUR F. ENNIS,  
H. D. JAMISON.